

## UNITED STATES PATENT OFFICE

GIOVANNI TAGLIANI, OF BASEL, SWITZERLAND, ASSIGNOR TO THE FIRM: CHEMICAL WORKS FORMERLY SANDOZ, OF BASEL, SWITZERLAND

## PROCESS FOR TREATING CELLULOSIC FIBERS WITH ALKALI

No Drawing. Application filed September 7, 1927, Serial No. 218,109, and in Germany October 29, 1926.

Various attempts have been made to improve the alkaline treatment of natural and artificial cellulosic fibers, such as is realized for instance in the mercerizing process, by the use of convenient admixtures. Soaps, sulphuricinoleic acids, alcohols and other substances have been proposed for this purpose. These admixtures have only little effect, so that large quantities are necessary to obtain a satisfactory result, which renders the process expensive. For instance, 20—30% of alcohol, calculated on the mercerizing lye, is necessary to mercerize satisfactorily a raw and sized cotton fabric without a previous bowking.

It has unexpectedly been found that this process can be considerably improved, if small quantities of a suitable mixture of phenolic substances and hydrogenated aromatic substances are added to the mercerizing lye, the action of the alkali is then quicker and more uniform. By the aid of these admixtures it is possible to mercerize raw and sized cotton fabrics without previous bowking.

These fabrics would otherwise not produce uniform effects without a previous bowking.

The addition of phenol alone to mercerizing lyes is already known. According to the U. S. specification 1,343,139 textile fabrics composed of mercerizable cellulosic fibers intermixed with artificial silk filaments of viscose are mercerized with a lye containing 5% of phenol. This addition has the only object to allow the performance of the mercerization of the cellulosic fiber without injury to the viscose silk, because, as is proved by many tests, phenol as well as its homologues do not affect at all the mercerizing operation of ordinary cotton.

The hydrogenated aromatic compounds being entirely insoluble in the concentrated alkaline lyes used for mercerization would not by themselves improve the process. But if they are used jointly with phenols as set forth above they act as very good wetting-out agents and greatly improve the wetting-out capacity of the alkaline lyes. This remarkably good action is based on the fact that the alkali phenolates formed in the mercerizing lye act as solvent and dispersing agent for the hydrogenated

aromatic compounds so as to allow to practically utilize their excellent wetting-out action.

The following hydrogenated aromatic substances come into consideration for the present process: The products of hydrogenation of naphthalene, naphthols and phenols, as for instance tetrahydro- and decahydronaphthalene, hydrogenated naphthols, cyclohexanol, methylcyclohexanols and mixtures of these substances. As phenolic substances, ordinary phenol, then especially the cresols and mixtures of them, further the higher phenol homologues may be used.

Mixtures of 2—12% of hydrogenated aromatic substances with 98—88% of phenols are most suitable for carrying out the new process, but this does not mean that mixtures of other proportions would be useless.

The effect of these admixtures is obtained even with small quantities (1—2% of the weight of the mercerizing lye). It consists in an increase of the wetting properties of the cellulosic fibers to an unexpected degree. This strong increase is the more unexpected as neither the phenols nor the hydrogenated aromatic substances by themselves cause appreciable increase of the wetting properties; only mixtures of such substances have this effect. The increase of the wetting properties of the fibers results not only in a quicker action of the alkali, but also in a more uniform effect.

## Example 1

A raw and unbowked cotton fabric is mercerized with a caustic soda lye of 34° Bé. to which 1½% of a mixture of 91% of a cresol mixture and 9% of a methylcyclohexanol mixture are added. The irregularities of the effect as obtained when the same fabric is mercerized with the same lye but without the above admixture, cannot be observed. The fabric shows a better lustre, an increased elasticity together with a deeper mercerization than that mercerized according to the old mercerizing process. Further the operation is carried out in a shorter time than is the case without the admixture.

*Example 2*

If 1½% of a mixture of 95% of cresols and 5% of tetrahydronaphthalene is added to a mercerizing lye of 36° Bé. the same effect as described in Example 1 is observed.

*Example 3*

A viscose fabric containing fibers which have been produced in different manufacturing operations is passed through a mercerizing lye of 20° Bé. to which 1½% (calculated on the weight of the lye) of a mixture of 90% of a cresol mixture and 10% of methylcyclohexanol mixture are added. The fabric is then squeezed out. The fabric thus treated can be dyed in more even shades than without this treatment.

What I claim is:

1. An improved process for the treatment of natural and artificial cellulose fibers with alkali, consisting in adding a mixture of a phenol and hydrogenated aromatic substances to the alkaline medium.
2. An improved process for the treatment of natural and artificial cellulosic fibers with alkali, consisting in adding a mixture of a cresol mixture and a methylcyclohexanol mixture to the alkaline medium.
3. An improved process for the treatment of natural and artificial cellulosic fibers with alkali, consisting in adding a mixture of 2-12% of hydrogenated aromatic substances and of 98-88% of phenolic substances to the alkaline lye, said mixture being added in quantities of 1-2% reckoned on the weight of the lye.

In witness whereof I have hereunto signed my name this 25th day of August 1927.

GIOVANNI TAGLIANI.

40

45

50

55

60

65